

# UNITED STATES PATENT OFFICE.

GEORGE STEELE DUNCAN AND GEORGE HENRY POTTS, OF EDINBURGH,  
SCOTLAND, ASSIGNORS TO AMERICAN OFFSET COMPANY, OF NEW  
YORK, N. Y., A CORPORATION OF NEW YORK.

## COMPOSITION FOR PREVENTING SET-OFFS IN PRINTING.

No. 828,673.

Specification of Letters Patent.

Patented June 19, 1906.

Application filed May 8, 1905. Serial No. 259,374.

*To all whom it may concern:*

Be it known that we, GEORGE STEELE DUNCAN and GEORGE HENRY POTTS, subjects of the King of the United Kingdom of Great Britain and Ireland, residing at Edinburgh, Scotland, have invented certain new and useful Improvements in Compositions for Preventing Set-Offs in Printing, of which the following is a specification.

10 This invention has for its object to provide an improved composition to prevent "set-off" or transfer of ink from one sheet to another or from one side to the reverse side of a sheet in printing, the said composition being particularly applicable for use in rotary printing-presses, rotary presses for magazine-printing, perfecting-machines, and flat-bed single-cylinder machines.

20 This invention in its preferred embodiment consists of a liquid composition which is particularly designed to be used for dampening the set-off rollers of printing-presses, although it is adapted for use in any manner for which "anti-set-off" compositions are or-

25 may be used.

The composition comprises in its preferred embodiment soap, preferably soft soap, a resinous substance, preferably turpentine, a non-volatile oil, preferably a non-drying oil, 30 such as olive-oil, a non-volatile oxidizing-oil, preferably boiled linseed-oil, a stable lubricating-oil, preferably neat's-foot oil, a highly-volatile mineral solvent, preferably naphtha, and an organic solvent, preferably 35 methylated spirits. The proportions in which we prefer to mix the above-named ingredients are as follows: equal volumes of each of the oils, that is to say, equal volumes of neat's-foot oil and boiled linseed-oil, 40 equal volumes of methylated spirits and naphtha, the volume of each of these being about half the volume of the boiled linseed-oil. The volume of the turpentine is preferably kept a little less than half the volume of 45 the boiled linseed-oil. The soap should be present in a proportion of about one pound to every four quarts of turpentine.

While the ingredients and proportions above given are those which are preferred, it 50 is to be understood that this invention is not limited thereto, as the proportions may be varied within wide limits and certain of the ingredients omitted and equivalents of the

ingredients substituted in their place. The invention is to be considered as broadly embracing the features of novelty in a composition for the purpose specified, as defined within the scope of the appended claims.

Among the changes which may be made in this composition without departing from the spirit of the invention or materially sacrificing the advantages thereof may be mentioned the following, which are, however, to be considered as merely illustrating a few of the many changes which the skill and experience of workers in the art will naturally suggest: The neat's-foot oil and the olive-oil are practically interchangeable—that is to say, one may be more or less completely replaced by the other. In place of the naphtha benzene or other similar volatile solvent may be used, but naphtha is preferred. The proportion of the boiled linseed-oil may be widely varied; but the best results have been obtained when the proportion of this ingredient is not diminished nor increased by more than one-third of the proportion indicated above. The proportion of the methylated spirits or naphtha, or both of these, may be very considerably increased without seriously affecting the character of the liquid, and the proportion of the naphtha may be materially diminished without impairing the usefulness of the liquid. The proportion of the soap may be materially varied, and where the composition is to be used with rotary machines it can be advantageously materially increased. Where the proportion of the soap is increased, it has been found that the best results are obtained by correspondingly increasing the proportion of the naphtha.

In preparing the composition, as it is desirable to apply heat to bring about as good an admixture of the soap as possible, it is preferable to defer adding the naphtha until after this heating and to take only one-third of the total volume of the liquid previous to the addition of the naphtha and to this third add the soap and stir well, gradually raising the temperature to about 130° Fahrenheit, then turn off the heat and allow the liquid to cool under gentle stirring. When the liquid is cool, add it to the remaining two-thirds, to which in the meantime naphtha has been added.

The liquid is preferably applied by a cloth

saturated with it and the principal lubricating-roller thereby given a good soaking. The frequency of the applications of the liquids for a given quantity of work depends largely

- 5 on the quality of the ink. With a rotary machine, if good ink is used, the initial dampening will suffice during the running of the reel, whereas with inferior ink the same machine and the same work may require a further application of the liquid when only half the reel is run.

Having thus described our invention, what we claim, and desire to secure by Letters Patent, is—

- 15 1. A composition for preventing "set-off" comprising a non-volatile oil and a resinous substance.  
 2. A composition for preventing "set-off" comprising olive-oil and a resinous liquid.  
 20 3. A composition for preventing "set-off" comprising a non-volatile oil and turpentine.  
 4. A composition for preventing "set-off" comprising an oil, a resinous substance, soap and a solvent of soap.  
 25 5. A composition for preventing "set-off" comprising an oil, a resinous substance, soap and a volatile solvent.  
 6. A composition for preventing "set-off" comprising an oil, a resinous liquid, soap and 30 naphtha.  
 7. A composition for preventing "set-off" comprising a non-volatile oil, turpentine, soap and a volatile solvent.  
 8. A composition for preventing "set-off" 35 comprising a non-volatile oil, turpentine, soap and a volatile mineral solvent.  
 9. A composition for preventing "set-off" comprising a non-volatile oil, a resinous substance, soap, a solvent of soap and an oxidizing-oil.  
 40 10. A composition for preventing "set-off" comprising a non-volatile oil, a resinous liquid, soap, a solvent of soap and linseed-oil.

11. A composition for preventing "set-off" comprising a non-volatile oil, turpentine, 45 soap, a volatile mineral solvent and boiled linseed-oil.

12. A composition for preventing "set-off" comprising a non-drying oil, a resinous substance, soap, a volatile solvent, an oxidizing-oil and a stable lubricating-oil. 50

13. A composition for preventing "set-off" comprising a non-drying oil, a resinous substance, soap, a volatile solvent, an oxidizing-oil and neat's-foot oil. 55

14. A composition for preventing "set-off" comprising a non-volatile oil, turpentine, soap, a volatile mineral solvent, boiled linseed-oil and neat's-foot oil.

15. A composition for preventing "set-off" 60 comprising a non-volatile oil, a resinous liquid, soap, a volatile mineral solvent, an oxidizing-oil, a stable lubricating-oil and an organic solvent.

16. A composition for preventing "set-off" 65 comprising a non-volatile oil, a resinous liquid, soap, a volatile mineral solvent, an oxidizing-oil, a stable lubricating-oil and methylated spirits.

17. A composition for preventing "set-off" 70 comprising a non-drying oil, turpentine, soap, a volatile solvent, linseed-oil, neat's-foot oil and an organic solvent.

18. A composition for preventing "set-off" 75 comprising olive-oil, turpentine, soap, naphtha, boiled linseed-oil, neat's-foot oil and methylated spirits, in substantially the proportions specified.

In testimony whereof we have signed our names to this specification in the presence of 80 two subscribing witnesses.

GEORGE STEELE DUNCAN.  
 GEORGE HENRY POTTS.

Witnesses:

WALLACE FAIRWEATHER,  
 JNO. ARMSTRONG, Junr.